

# UNITED STATES PATENT OFFICE.

FREDERICK LEE, OF NORWICH, ENGLAND, ASSIGNOR TO GEORGE EMANUEL HALDIN-STEIN, OF NORWICH, ENGLAND.

## SOLUTION FOR USE IN THE MANUFACTURE OF BOOTS AND SHOES.

1,410,685.

Specification of Letters Patent. Patented Mar. 28, 1922.

No Drawing.

Application filed May 25, 1920. Serial No. 384,191.

*To all whom it may concern:*

Be it known that I, FREDERICK LEE, a subject of the King of Great Britain, residing at 37 Aylsham Road, Norwich, in the county of Norfolk, England, have invented certain new and useful Improvements in a Solution for Use in the Manufacture of Boots and Shoes, of which the following is a specification.

10 This invention relates to a solution for use in the manufacture of boots and shoes and is particularly intended for use in attaching the soles and heels to the uppers without the use of nails or similar fastening

15 means.

According to the invention the solution consists of balata and naphtha made up of

the following ingredients mixed together in any appropriate manner in or about the portions stated, viz:—

20 15 ounces of Venezuelan balata.

20 ounces of Tumaco block balata.

15 ounces of solvent naphtha.

What I claim and desire to secure by Letters Patent of the United States is:—

25 1. An adhesive solution consisting of Venezuelan balata and Tumaco block balata dissolved in solvent naphtha.

2. A solution for use in attaching the soles and heels of boots and shoes to their uppers 30 consisting of about 15 ounces of Venezuelan balata, about 20 ounces of Tumaco balata and about 15 ounces of solvent naphtha.

FREDERICK LEE.